

Dec. 1, 1931.

H. BÖVING

1,834,376

INSULATED WIRE

Filed June 20, 1924



Inventor:  
Henrik Böving,  
by *E.W. Adams Atty*

## UNITED STATES PATENT OFFICE

HENRIK BÖVING, OF NEW YORK, N. Y., ASSIGNOR TO WESTERN ELECTRIC COMPANY,  
INCORPORATED, OF NEW YORK, N. Y., A CORPORATION OF NEW YORK

## INSULATED WIRE

Application filed June 30, 1924. Serial No. 721,370.

This invention relates to electrically insulated wire and particularly to improvements in so-called "flame-proof" electrically-insulated wire.

The object of the invention is to provide a flame-proof insulated wire which will be highly efficient in service and economical in manufacture.

A feature of the invention is a wire having an insulating covering, such as rubber, rubber-containing materials or enamel, and a coating of sodium silicate or commercial "water-glass" applied thereon.

A further feature is a wire having an insulating covering, a coating of sodium silicate or water-glass applied over the insulating covering and an exterior textile covering.

A further feature is a wire having an insulating covering, a coating of sodium silicate or water-glass applied on the insulating covering, and an exterior covering of flame-proofed cotton.

A further feature is a wire having a rubber-insulation covering, a coating comprising a mixture of sodium silicate or water-glass and glycerine or the equivalent applied thereon, and an exterior covering comprising flame-proofed cotton.

The single figure shows an insulated wire embodying one form of the invention.

Referring to the figure, the insulated wire comprises a core 1 of electrically conducting material, a coating 2 of rubber or other insulating material applied over the core, a second coating 3 of flame-proof material, such as sodium silicate or water glass, applied over the insulating coating 2, and an exterior textile covering 4, such as braided cotton or flame-proofed cotton, applied over the flame-proof coating 3.

One way of producing the flame-proof insulated wire embodying the invention is to pass a wire of electrically-conducting material having an insulation covering such as rubber, rubber compounds, or enamel, through a solution of sodium silicate or what is known commercially as "water-glass", the solution being of the proper consistency to give the required thickness of coating. The wire may be drawn through the solution in

any suitable manner, but, preferably, should be drawn out of the solution in a vertical direction so as to obtain a coating of uniform thickness around the wire. When the wire is withdrawn from the solution, after a short interval of drying, 5 or 6 minutes is sufficient, the material will be set so that a uniform coating 3 of the dried sodium silicate or water-glass will be obtained on the rubber-covered wire. The flexibility and adherence of the coating will be sufficient so that the wire may be reeled or so that it will stand the customary amount of handling in the braiding process to follow.

If desired, a more flexible and more adhesive coating may be obtained without materially decreasing its flame-proofing qualities by adding about 10 per cent of glycerine or the equivalent to the solution of sodium silicate or water-glass through which the rubber-covered wire is drawn.

The flame-proof coating of sodium silicate, water-glass or mixtures of those materials with glycerine, may be further protected from abrasion and vibration by applying an outer textile covering 4, preferably cotton or cotton braid, over it by any of the processes well-known in the art. An additional flame-proof and water-proof protection may be obtained by impregnating the textile fabric with any suitable flame-proofing material, for example, sodium magnesium borate.

If desired, the textile serving 4 may be applied before the water glass coating has dried, so that the coating in its liquid or partially set condition is taken up to some extent by the serving. In either case the water glass is effectively prevented by the serving from flaking off or from being rubbed off or otherwise lost or displaced from handling or bending of the wire. A practically continuous coating of the water glass is thus maintained over the insulation coating.

The product obtained by the above-described process, comprising an insulated wire having a coating of sodium silicate, water-glass, or mixtures thereof with glycerine, applied over the insulating coating, and an outer textile covering or flame-proofed textile covering has been found to provide an effi-

cient flame-proof conductor. In fact, it has been found that if wire constructed in this manner is held in a fire of sufficiently intense heat until the insulation is burning briskly, upon removal of the source of the heat, the flame will almost immediately die down.

Such wire has a practical application as "jumper" wire used in distributing frames in telephone central stations. However, it is 10 not restricted to such use, but may be used in any other situation where flame-proofing is necessary.

What is claimed is:

1. An insulated wire comprising a core of 15 electrically conducting material having a coating of rubber insulating material, a second coating of sodium silicate applied immediately over said first-mentioned coating, and a cotton covering impregnated with 20 flame-proofing material applied over said coating of sodium silicate.
  2. A flame-proofed insulated conductor comprising a rubber-insulated wire, a coating of water-glass applied immediately thereover, and a textile serving applied over the water-glass of sufficiently close texture and fit, to hold the water-glass in place during use of the wire.
  3. A wire having an electrical insulation 25 of rubber, a flame-proof insulation of dried water-glass applied immediately over the rubber, and a mechanical insulation of closely woven cotton over the dried water-glass.
  4. An insulated wire comprising a core of 30 electrically conducting material having a coating of rubber insulating material applied immediately thereover, a second coating containing sodium silicate and glycerine applied over said coating of rubber insulating 35 material, and a cotton covering impregnated with flame-proofing material applied over said second coating.
  5. An insulated wire comprising a core of 40 electrically conducting material having a coating of rubber insulating material applied immediately thereover, a second coating containing water-glass and glycerine applied over said coating of rubber insulation, and a flame-proofed cotton serving over the whole.
- 50 In witness whereof, I hereunto subscribe my name this 20th day of June, A. D. 1924.

HENRIK BÖVING.